

## 1

3,513,094

## LUBRICANT COMPOSITIONS

Homer H. Farmer, Westport, Harold F. Tompkins, Trumbull, and Bobby W. Malone, Norwalk, Conn., assignors to R. T. Vanderbilt Company, Inc., New York, N.Y., a corporation of New York  
No Drawing. Filed Apr. 26, 1967, Ser. No. 633,677  
Int. Cl. C10m 1/48

U.S. Cl. 252—32.7

8 Claims

## ABSTRACT OF THE DISCLOSURE

An improved extreme pressure lubricant combining an antimony dihydrocarbylphosphorodithioate with a second, known extreme pressure or wear inhibiting agent, such as chlorinated paraffin, sulfurized oil, a lead dithiocarbamate or lead naphthenate, in a lubricating oil or lubricating grease base.

This invention relates to improved lubricant compositions, and more particularly to lubricant compositions containing antimony dihydrocarbylphosphorodithioates combined with other wear inhibitors and extreme pressure agents in a lubricating oil base.

There are several types of gears and bearings, such as hypoid gears and heavily loaded bearings, wherein it is extremely difficult to maintain a thin film of lubricant between the gear or bearing surfaces. When the film of lubricant ruptures, the high spots on the surfaces where metal-to-metal contact occurs become deformed. The friction increases to cause localized welding. As the weld is sheared by the relative motion of the surfaces, particles of metal are removed. The contacting surfaces become rough and pitted, and they eventually fail by seizing or scoring.

The special types of lubricants developed for use under these conditions are known as extreme pressure (E.P.) lubricants. E.P. lubricants are prepared by adding special E.P. agents to lubricating oils or greases. Other antiwear and anticorrosion agents are often added to prepare a lubricant with several desirable special properties.

It has been proposed heretofore to add various metallic salts of dihydrocarbyl esters of phosphorodithioic acids as E.P. agents and wear inhibitors to lubricating oils or greases in order to prepare E.P. and antiwear lubricating compositions. Many of these proposed E.P. lubricants have exhibited only moderately acceptable E.P. and antiwear properties.

It is therefore an object of the present invention to provide improved lubricating compositions exhibiting highly effective extreme pressure and antiwear properties.

According to the invention it has been found that antimony dihydrocarbylphosphorodithioates combined with other well-known E.P. and antiwear agents in lubricating oils and greases exhibit surprising and unexpected synergistic E.P. and antiwear properties. The lubricating compositions of the invention are suitable for use on heavily loaded surfaces where extreme pressure conditions prevail to prevent scuffing and seizure of engaging movable parts. Examples of the suitable uses include gear oils, crankcase oils, cutting oils, metal working lubricants, hydraulic fluids and automatic transmission fluids.

The antimony dihydrocarbylphosphorodithioates used in the invention have the structural formula:



## 2

wherein R is a hydrocarbyl radical selected from the group consisting of (A) lower alkyl radicals containing from two to eight carbon atoms, such as ethyl, n-propyl, i-propyl, n-butyl, i-butyl, sec.-butyl, tert.-butyl, amyl, n-hexyl, i-hexyl, n-heptyl, n-octyl, i-octyl, and 2-ethylhexyl; (B) substituted and unsubstituted cycloalkyl radicals containing five or six carbon atom rings, with the substituted cycloalkyls containing at least one of the lower alkyl radicals, e.g., cyclopentyl, methylcyclopentyl, cyclohexyl, methyl cyclohexyl and ethylcyclohexyl; and (C) substituted and unsubstituted phenyl radicals with the substituted phenyl radicals containing at least one of the substituents selected from the group consisting of alkyl radicals containing from one to nine carbon atoms. Examples of the substituted phenyl radicals include cresyl, tolyl, ethylphenyl, propylphenyl, butylphenyl, amylphenyl, octylphenyl and nonylphenyl groups.

The other E.P. and antiwear additives operable in the invention include the well-known E.P. agents, exemplified by lead naphthenate, halogenated paraffin, sulfurized fatty oils, and metal dialkyldithiocarbamates, wherein the metals include molybdenum, antimony, cadmium, zinc and lead, and the alkyl groups range from C<sub>1</sub> to C<sub>20</sub>.

The ratios of the amounts of antimony dihydrocarbylphosphorodithioates to other E.P. additives vary with the type of supplemental E.P. additive employed, as well as with the length of the hydrocarbyl group in the antimony dihydrocarbylphosphorodithioates. It has been found, however, that as low as 0.2% antimony dihydrocarbylphosphorodithioate and 0.4% supplemental E.P. additives will provide significant synergistic levels of E.P. performance.

The lubricating oil base stock used in preparing the lubricating composition may be straight mineral lubricating oils, distillates, greases, bright stock residua, etc. Synthetic lubricating oils, such as hydrogenated oils, glycol ethers, dibasic acid esters, and other polyester and polyether synthetic lubricating oils can also be used, as can mixtures of the synthetic oils. It is also possible to employ mixtures of synthetic oils and petroleum base mineral oils as the base.

The lubricating compositions may contain other components if desired, such as dispersing agents, rust inhibitors, antioxidants, and pour depressants.

In the following examples, the antimony dihydrocarbylphosphorodithioates were prepared by conventional means. The examples are intended to illustrate the properties of the lubricating compositions, including both oils and greases, as described in this specification, and are not intended to limit in any way the scope of the invention.

## EXAMPLE 1

Timken Load-Bearing Test using antimony di-n-propylphosphorodithioate and chlorinated paraffin

To separate portions of a representative solvent-refined, hydro-treated, high viscosity index, SAE 90 Mid-Continent base oil were added: 0.25% by weight of chlorinated paraffin (described as containing 42.45% combined chlorine and having a specific gravity of 1.165–1.210 and an SUS viscosity at 210° F. of 184–192 seconds); 1.0% chlorinated paraffin; 0.75% antimony di-n-propylphosphorodithioate; 1% antimony di-n-propylphosphorodithioate; a combination of 0.25% chlorinated paraffin and 0.75% of the antimony phosphorodithioate; and a combination of 0.1% chlorinated paraffin and 0.3% of the antimony phosphorodithioate. An untreated portion of the base oil served as a control.

The lubricating compositions so produced were subjected to the Timken Load-Bearing Test in the Timken Lubricant Tester in which a hardened steel ring rotating at 800 r.p.m. was flooded by the test lubricant at 100° F.

while a hardened steel block was pressed against it by a system of weights and levers. The highest weight which did not produce scoring of the block in 10 minutes running time was recorded as the passing load or O.K. load, which is a recognized measure of the load-carrying capacity of the lubricant. The values obtained in accordance with this standard test are set forth in Table I below.

TABLE I

| SAE 90 base oil containing    |                                           | Timken O.K. load, lbs. |          |            |
|-------------------------------|-------------------------------------------|------------------------|----------|------------|
| Chlorinated paraffin, percent | Sb di-n-propylphosphorodithioate, percent | Observed               | Observed | Calculated |
| 0.....                        | 0.....                                    | 0.....                 | 7.....   | .....      |
| 0.25.....                     | 0.....                                    | 0.....                 | 10.....  | 3.....     |
| 1.0.....                      | 0.....                                    | 0.....                 | 25.....  | 18.....    |
| 0.....                        | 0.75.....                                 | 0.....                 | 35.....  | 28.....    |
| 0.....                        | 1.0.....                                  | 0.....                 | 55.....  | 48.....    |
| 0.1.....                      | 0.3.....                                  | 0.....                 | 25.....  | 18.....    |
| 0.25.....                     | 0.75.....                                 | 0.....                 | 75.....  | 68.....    |

These data show that the observed load increase for the combination of 0.25% chlorinated paraffin and 0.75% antimony phosphorodithioate was 68 lbs.; whereas the calculated increase is 31 lbs., which is less than one-half the observed increase. The observed load increase for 0.1% chlorinated paraffin and 0.3% antimony phosphorodithioate was 18 lbs., and the calculated increase is 12 lbs. which is two-thirds the observed increase.

## EXAMPLE 2

Timken Load-Bearing Test using, antimony bis(2-ethylhexyl)phosphorodithioate and chlorinated paraffin

To separate portions of the base oil described in Example 1 were added 0.4% by weight of chlorinated paraffin, 2% by weight of antimony bis(2-ethylhexyl)phosphorodithioate, and a combination of 0.4% of chlorinated paraffin and 2% of antimony bis(2-ethylhexyl)phosphorodithioate. An untreated portion of the base oil served as a control. The lubricating compositions so produced were subjected to the Timken Load-Bearing Test with the following results:

TABLE II

| SAE 90 base oil containing    |                                                  | Timken O.K. load, lbs. |          |            |
|-------------------------------|--------------------------------------------------|------------------------|----------|------------|
| Chlorinated paraffin, percent | Sb bis(2-ethylhexyl)-phosphorodithioate, percent | Observed               | Observed | Calculated |
| 0.....                        | 0.....                                           | 0.....                 | 7.....   | .....      |
| 0.4.....                      | 0.....                                           | 0.....                 | 13.....  | 6.....     |
| 0.....                        | 2.0.....                                         | 0.....                 | 40.....  | 33.....    |
| 0.4.....                      | 2.0.....                                         | 0.....                 | 65.....  | 58.....    |

These data show that the actual increase in load-bearing capacity of the oil containing the combination of chlorinated paraffin and the antimony phosphorodithioate (58 lb. over that of the base oil) is far in excess of that which could be expected from additive effect alone (39 lbs. over base oil).

## EXAMPLE 3

Timken Load-Bearing Test using antimony di-n-propylphosphorodithioate and lead naphthenate

To separate portions of the base oil described in Example 1 were added 1.5% by weight of light colored lead naphthenate (containing 30% lead), 0.75% antimony di-n-propylphosphorodithioate, a combination of 1.5% lead naphthenate and 0.75% antimony di-n-propylphosphorodithioate, and a combination of 0.4% lead naphthenate and 0.2% of the antimony phosphorodithioate. An untreated portion of the base oil served as the control. The lubricating compositions thus formed were subjected

to the Timken Load-Bearing Test with the results tabulated below.

TABLE III

| 5  | SAE 90 base oil containing |                                           | Timken O.K. load, lbs. |          |            |
|----|----------------------------|-------------------------------------------|------------------------|----------|------------|
|    | Lead naphthenate, percent  | Sb di-n-propylphosphorodithioate, percent | Observed               | Observed | Calculated |
| 10 | 0.....                     | 0.....                                    | 0.....                 | 7.....   | .....      |
|    | 1.5.....                   | 0.....                                    | 15.....                | 8.....   | .....      |
|    | 0.....                     | 0.75.....                                 | 35.....                | 28.....  | .....      |
|    | 0.4.....                   | 0.2.....                                  | 50.....                | 43.....  | 11.....    |
|    | 1.5.....                   | 0.75.....                                 | 80.....                | 73.....  | 36.....    |

15 Thus it is shown that the O.K. load of oil containing both of the additives is increased twice as much (73 lbs.) as could be expected on the basis of additives effect alone (36 lbs.).

## EXAMPLE 4

20 4-Ball Weld Load Test using antimony bis(2-ethylhexyl)-phosphorodithioate and lead naphthenate

To separate portions of the oil described in Example 1 were added: 1.5% by weight of lead naphthenate; 25 3.0% by weight of antimony bis(2-ethylhexyl)phosphorodithioate; a combination of 1.5% lead naphthenate and 3.0% antimony bis(2-ethylhexyl)phosphorodithioate; and a combination of 0.5% lead naphthenate and 1.0% antimony bis(2-ethylhexyl)phosphorodithioate. An untreated portion of the oil served as a control. The compositions thus prepared were subjected to the 4-Ball Weld Load Test in which a  $\frac{1}{2}$ -inch steel ball is rotated in contact with three similar balls which are clamped in a stationary position so as to provide three points of contact. The balls are bathed in lubricating composition at room temperature, and increasing loads are applied for ten seconds each to the ball rotating at 1800 r.p.m. The load at which the balls weld together is recorded. The results of these tests are reported below.

TABLE IV

| 45 | SAE 90 base oil containing |                                                  | 4-ball weld load, Kg. |          |            |
|----|----------------------------|--------------------------------------------------|-----------------------|----------|------------|
|    | Lead naphthenate, percent  | Sb bis(2-ethylhexyl)-phosphorodithioate, percent | Observed              | Observed | Calculated |
| 50 | 0.....                     | 0.....                                           | 105.....              | .....    | .....      |
|    | 1.5.....                   | 0.....                                           | 140.....              | 35.....  | .....      |
|    | 0.....                     | 3.0.....                                         | 215.....              | 110..... | .....      |
|    | 1.5.....                   | 3.0.....                                         | 330.....              | 225..... | 145.....   |
|    | 0.5.....                   | 1.0.....                                         | 215.....              | 110..... | 48.....    |

These data show that there is a far greater than additive effect on the 4-Ball Weld Load when 1.5% lead naphthenate and 3.0% antimony bis(2-ethylhexyl)-phosphorodithioate are used together than when used alone. The expected increase was 35 kg. due to lead naphthenate and 110 kg. due to the phosphorodithioate, a total of 145 kg. while the actual increase was 225 kg.

60 When the quantities of each of these additives were cut to one-third, the expected increase would be one-third that expected from the original combination of one-third of 145, or 48 kg. Thus is illustrated one of the common methods for determining synergism, i.e., measuring the effect of the separate components at given concentrations, then comparing the expected additive effect with that actually obtained by combinations containing decreased quantities of the separate components.

From the values shown in the third and last lines of 70 Table IV it is obvious that due to the synergistic effect the high increase in weld load due to the antimony phosphorodithioate above can be maintained by substituting a large part of it with the much less expensive lead naphthenate. (A decrease from 3.0% to 1.0% phosphorodithioate.)

**5**  
**EXAMPLE 5**

4-Ball Weld Load Test using antimony di(nonylphenyl) phosphorodithioate and sulfurized sperm oil in a mineral oil base grease

To separate portions of a lithium 12-hydroxy-stearate mineral oil base grease were added: 1% by weight of sulfurized sperm oil (10% sulfur); 2% of antimony di(nonylphenyl) phosphorodithioate; and a combination of 1% sulfurized sperm oil and 2% antimony di(nonylphenyl) phosphorodithioate. Another portion of the grease served as an untreated control. The compositions thus obtained were subjected to the 4-Ball Weld Load Test described in Example 4 in which grease was substituted for the lubricating oil in the cup in which the balls are held. The weld loads obtained are tabulated below:

TABLE V

| Lithium grease containing—    |                                                | 4-ball weld load, kg. |          |          |
|-------------------------------|------------------------------------------------|-----------------------|----------|----------|
| Sulfurized sperm oil, percent | Sb di(nonylphenyl) phosphorodithioate, percent | Observed              | Observed | Increase |
| 0-----                        | 0                                              | 120                   | -----    | -----    |
| 1.0-----                      | 1.0                                            | 130                   | 10       | -----    |
| 0-----                        | 2.0                                            | 180                   | 40       | -----    |
| 1.0-----                      | 2.0                                            | 210                   | 90       | 50       |

Thus it is shown that far more than additive effect was obtained when the two E.P. agents, sulfurized sperm oil and antimony di(nonylphenyl) phosphorodithioate were present in combination in a lithium grease. This cooperation between the two E.P. agents was unexpected, and it amounted to almost double the calculated increase in weld load (90 kg. as opposed to 50 kg.).

## EXAMPLE 6

Timken Load-Bearing Test using antimony di-n-propyl phosphorodithioate and lead naphthenate in a grease

To separate portions of an aluminum complex mineral oil base lubricating grease were added: 1.5% by weight of lead naphthenate; 0.75% of antimony di-n-propyl phosphorodithioate; 1.0% of antimony di-n-propyl phosphorodithioate; a combination of 1.5% lead naphthenate and 0.75% antimony di-n-propyl phosphorodithioate; and a combination of 1.0% lead naphthenate and 0.5% antimony di-n-propyl phosphorodithioate. An untreated portion of the aluminum complex grease served as control. The compositions thus prepared were subjected to the Timken O.K. Load Test described in Example 1 modified by pumping the test grease against the ring and block at the rate of about 1.5 ounces of grease per minute. The results of these tests are tabulated below:

TABLE VI

| Aluminum Complex Grease Containing |                                           | Timken O.K. load, lbs. |          |          |
|------------------------------------|-------------------------------------------|------------------------|----------|----------|
| Lead naphthenate percent           | Sb di-n-propyl phosphorodithioate percent | Observed               | Observed | Increase |
| 0-----                             | 0                                         | 10                     | 5        | -----    |
| 1.5-----                           | 0                                         | 15                     | 5        | -----    |
| 0-----                             | 0.75                                      | 25                     | 15       | -----    |
| 1.5-----                           | 0.75                                      | 60                     | 50       | 20       |
| 1.0-----                           | 0.5                                       | 35                     | 25       | 14       |

It is thus shown that far more than additive effect was obtained when 1.5% lead naphthenate and 0.75% antimony phosphorodithioate were added to an aluminum complex grease. An increase of 50 pounds in Timken O.K. Load was observed compared with an expected additive increase of 20 pounds. When two-thirds of the amounts of additives were added, the observed increase in Timken O.K. Load, 25 pounds, was far greater than that calculated on the basis of an expected two-thirds increase. It was even larger than the increase calculated for the higher concentration (25 lbs. as opposed to 20 lbs.).

**6**  
**EXAMPLE 7**

4-Ball Weld Load Test using antimony bis(2-ethylhexyl) phosphorodithioate and lead diamyl dithiocarbamate

To separate portions of the base oil described in Example 1 were added: 2% by weight of lead diamyl dithiocarbamate; 3% by weight of antimony bis(2-ethylhexyl) phosphorodithioate; and a combination of 2% of the lead dithiocarbamate and 3% of the antimony phosphorodithioate. An untreated portion of the base oil served as a control. The lubricating compositions were subjected to a 4-Ball Weld Load Test with the following results:

15

TABLE VII

| SAE 90 base oil containing                       |                                      | 4-ball E.P. weld load, kg. |          |          |
|--------------------------------------------------|--------------------------------------|----------------------------|----------|----------|
| Sb bis(2-ethylhexyl)-phosphorodithioate, percent | Lead diamyl dithiocarbamate, percent | Observed                   | Observed | Increase |
| 0-----                                           | 0                                    | 105                        | -----    | -----    |
| 2.0-----                                         | 0                                    | 225                        | 120      | -----    |
| 0-----                                           | 3.0                                  | 215                        | 110      | -----    |
| 2.0-----                                         | 3.0                                  | 375                        | 270      | 230      |

25

These data show that the observed increase for the combination of 2.0% lead diamyl dithiocarbamate and 3.0% of the antimony phosphorodithioate was significantly in excess of the calculated increase (270 kg. over 230 kg.).

We claim:

1. Lubricating compositions exhibiting synergistic extreme pressure and antiwear properties consisting essentially of (1) antimony dihydrocarbylphosphorodithioates, wherein the hydrocarbyl group is selected from the group consisting of (A) alkyl radicals containing from two to eight carbon atoms, and (B) substituted and unsubstituted phenyl radicals with the substituted radicals containing at least one substituent selected from the group consisting of alkyl radicals containing from one to nine carbon atoms; (2) one or more extreme pressure agents selected from the group consisting of lead naphthenate, halogenated paraffin, sulfurized fatty oils and metal dialkyldithiocarbamates, wherein the alkyl groups have a chain length of from one to twenty carbon atoms; and (3) a lubricating base selected from the group consisting of lubricating oil and lubricating grease bases.

2. A lubricating composition as described in claim 1, wherein the phosphorodithioate is antimony di-n-propyl phosphorodithioate, and the second extreme pressure agent is chlorinated paraffin.

3. A lubricating composition as described in claim 1, wherein the phosphorodithioate is antimony bis(2-ethylhexyl)phosphorodithioate and the second extreme pressure agent is chlorinated paraffin.

4. A lubricating composition as described in claim 1, wherein the phosphorodithioate is antimony di-n-propyl phosphorodithioate and the second extreme pressure agent is lead naphthenate.

5. A lubricating composition as described in claim 1, wherein the phosphorodithioate is antimony bis(2-ethylhexyl)phosphorodithioate and the second extreme pressure agent is lead naphthenate.

6. A lubricating composition as described in claim 1, wherein the phosphorodithioate is antimony di(nonylphenyl)phosphorodithioate and the second extreme pressure agent is sulfurized sperm oil.

7. A lubricating composition as described in claim 1, wherein the phosphorodithioate is antimony di-n-propyl phosphorodithioate and the second extreme pressure agent is lead naphthenate.

8. A lubricating composition as described in claim 1, wherein the phosphorodithioate is antimony bis(2-ethyl-

3,513,094

7

hexyl)phosphorodithioate and the second extreme pressure agent is lead diamyldithiocarbamate.

8

2,976,122 3/1961 Ertelt.  
3,222,280 12/1965 Wolfram et al.  
3,269,946 8/1966 Wiese.

**References Cited**

**UNITED STATES PATENTS**

2,511,630 6/1950 Goren et al.  
2,773,860 12/1956 Musselman.

5 PATRICK P. GARVIN, Primary Examiner

W. J. SHINE, Assistant Examiner